

# UNITED STATES PATENT OFFICE.

EUGENE H. COWLES, OF CLEVELAND, OHIO.

## PROCESS OF MANUFACTURING IRON OR STEEL.

SPECIFICATION forming part of Letters Patent No. 397,491, dated February 12, 1889.

Application filed December 24, 1887. Serial No. 258,920. (No specimens.)

*To all whom it may concern:*

Be it known that I, EUGENE H. COWLES, of Cleveland, in the county of Cuyahoga and State of Ohio, have invented a certain new and 5 Improved Process of Manufacturing Iron or Steel; and I do hereby declare the following to be a full, clear, and exact description of the invention, such as will enable others skilled in the art to which it pertains to make and 10 use the same.

My invention relates to a new process of improving iron and steel; and it consists in steps hereinafter described and claimed.

It is well known that many metals when hot 15 have a great affinity for certain elements that exist in a gaseous state in the atmosphere to which they are exposed while in a molten condition. In the smelting and manufacture 20 of iron and steel oxygen appears to be the most noxious and injurious element encountered. When fluid, the iron takes up large quantities of oxygen, either in a free state or combined with other elements—such as carbon—and the oxygen or carbon oxide remains 25 in the metal either in mechanical mixture or in the state of chemical combination with the iron even after the metal has become cold. The worst effect of oxygen thus found in iron or steel is the formation of certain sub-oxides 30 of iron and the leaving of cavities through the mass, whose sides are lined with the sub-oxide or streaks, seams, fissures, and flaws in rolled or forged iron or steel which are caused by the non-welding character of the sub-oxide 35 that forms on the faces of these seams or cracks. The presence of the sub-oxide throughout mass of iron or steel in minute specks that can only be seen by the microscope likewise seriously impairs the strength, hot and 40 cold working qualities, and welding properties of iron and steel. In fact, it is susceptible of proof that the sub-oxide that forms in iron and steel is more disastrous to its value than the so-called "blow-holes." In order to 45 prevent these sub-oxides from forming and to eliminate as far as possible the bad effects of oxygen and other injurious elements—such, for instance, as sulphur—from iron or steel, I use an alloy of silicon and aluminium. 50 This alloy of aluminium and silicon is somewhat variable in its proportions; but it has been found that the silicon may form as high

as fifty percent of the alloy. If this alloy be added to iron or steel while in a fluid state, or melted together with iron or steel, or reduced directly from the ores of silicon and aluminium into iron or steel, it will remove nearly all the oxygen present. It may likewise be added to a bath of molten iron or steel in the form of an alloy of silicon, aluminium, 60 and iron or steel.

By the application of this invention and subsequent thereto many tons of iron or steel are now being refined and improved weekly in this country and abroad, and it is found 65 that it is a much cheaper process than that wherein pure aluminium or an alloy of aluminium and iron is used to effect a somewhat similar result. The preferable manner of using this invention is to treat a bath of iron 70 or steel while in the furnace or converter with a small percentage of aluminium and silicon alloy, or alloy of the same with iron, the same to contain not to exceed one-fifth of one per cent. of aluminium and silicon combined, the 75 same to be melted together with the iron or steel, in order to give the aluminium and silicon sufficient time to thoroughly mix with the entire mass of material to be treated. If the metal is immediately taken from the fire as 80 soon as the aluminium and silicon is well incorporated, the best results will be obtained; but should the heat be prolonged, and it is desired to take extra precautions, another five-hundredths of one per cent. of aluminium 85 and silicon combined may be added, alone or alloyed with iron, to the material, if it be still fluid after it leaves the furnace; but care should be taken to have the bath of molten metal to be treated superheated before leaving the furnace if an alloy of iron, silicon, and aluminium is to be used, as it has a very high melting-point, and without such superheating it may chill the bath of steel or iron to which 90 it is added.

I am fully aware that aluminium has heretofore frequently been added to iron and steel. It is claimed that traces of it have been found in "Wootz steel" and many other irons and steels; but these claims are of doubtful authenticity. Yet it has been frequently added to steel and iron in its pure state. Deville, Dr. Percy, and Sir Lothian Bell have all made alloys of iron and steel with pure aluminium;

and hence I do not claim an alloy of iron or steel and aluminium, nor methods of treating iron or steel with aluminium or alloy of aluminium and iron.

5 An alloy of silicon and aluminium is much more economic and produces better results than the use of aluminium alone or combined with iron.

In reducing silicon and aluminium to form

- 10 the desired alloy it is more convenient to add more or less iron for purpose of collecting these light materials in the furnace where they are reduced, and consequently such alloy of the three elements is more frequently used
- 15 in carrying out my invention than an alloy of silicon and aluminium alone.

What I claim is—

- 1. The herein-described step in the process of manufacturing iron and steel, consisting
- 20 in the admixture with the molten iron or steel of an alloy of silicon and aluminium in about the proportions specified, substantially as set forth.

2. The herein-described step in the process of manufacturing iron and steel, consisting 25 in melting together iron or steel with an alloy of silicon, aluminium, and iron, substantially as set forth.

3. The herein-described step in the process of manufacturing iron and steel, consisting 30 in melting together iron or steel with an alloy of silicon and aluminium.

4. The herein-described step in the process of manufacturing iron and steel, consisting 35 in the admixture with the molten iron or steel of an alloy of silicon, aluminium, and iron, substantially as set forth.

In testimony whereof I sign this specification, in the presence of two witnesses, this 21st day of December, 1887.

EUGENE H. COWLES.

Witnesses:

ALBERT E. LYNCH,  
CHAS. H. DORER.